

## UNITED STATES PATENT OFFICE

CHARLES WILFRED PALMER AND STEPHEN MILLER FULTON, OF SPONDON, NEAR DERBY, ENGLAND, ASSIGNORS TO CELANESE CORPORATION OF AMERICA, A CORPORATION OF DELAWARE

TREATMENT OF THREADS, FABRICS, OR OTHER MATERIALS COMPOSED OF OR CONTAINING ARTIFICIAL FILAMENTS

No Drawing. Application filed November 16, 1925, Serial No. 69,526, and in Great Britain May 26, 1925.

This invention relates to the treatment of threads, knitted woven or other fabrics or other materials composed of or containing filaments or fibres (hereinafter included in the term filaments) of cellulose acetate artificial silk, and in particular "dry-spun" cellulose acetate artificial silk.

When cellulose acetate artificial silk and particularly "dry-spun" cellulose acetate artificial silk made from cellulose acetate solutions of relatively low concentrations, is subjected to the action of hot or boiling solutions of acids or acid salts or hot or boiling water, particularly water between about 90° C. and the boiling point, or moist steam, the cellulose acetate artificial silk can lose its natural high lustre to a greater or less extent and become converted to a more or less delustrated condition.

20 The application of processes in which such delustring of cellulose acetate artificial silk occurs, for the production of threads or goods showing the effects of wool, hair or other modified effects, forms the subject of U. S.

25 Patent No. 1,554,801, according to which lustrous cellulose acetate filaments or threads, or goods containing the same, are subjected to the action of agents whereby the cellulose acetate filaments or fibres are delustrated to any 30 desired extent and more or less crinkled. The filaments or fibres of cellulose acetate resulting from such treatment of said patent are in fact "hollow" filaments, due probably to the action of the delustring and crinkling agents 35 in releasing in or from the filaments residual traces of solvent present in the filaments.

Some qualities of cellulose acetate artificial silk are much more resistant than others to delustring agencies, this resistance varying 40 with the quality of the cellulose acetate of which the threads or filaments are made and also with the concentration of the cellulose acetate solutions used for spinning the same. In particular, threads or filaments made with 45 very high quality cellulose acetates substantially undegraded in the cellulose molecule, are especially resistant to delustring agencies. Further, artificial silks spun from cellulose acetate solutions of high concentrations, e. g. 50 containing from 20 to 25 or 30% or more of

cellulose acetate, are not so liable to become delustrated as those produced from less concentrated solutions containing for example under about 10% or up to about 16 or 18% of cellulose acetate.

55 Delustring may, however, occur even with very resistant qualities of cellulose acetate artificial silk under the prolonged or especially intensive action of said agencies.

The object of the present invention is to provide means for preventing or controlling to any desired degree the delustring of cellulose acetate artificial silk caused by water or solutions, especially hot or boiling water or solutions, particularly acid solutions, moist steam or other aqueous agents or media. By means of the invention, the lustre of the acetyl cellulose threads or filaments exposed to such delustring agencies may be preserved wholly or may be modified to any desired degree according to the technical effect desired.

60 We have found that the presence of one or more protecting agents or substances restraints, retards or even prevents the delustring action of such agencies. The presence 65 of such protecting agents or substances enables any desired degree of protection of lustre to be afforded according to the protecting agent or substance used, the concentration thereof and the nature and duration of exposure to the aqueous media. Any agents having the desired protecting action may be employed for the purpose of the invention. Protecting agents we have found useful for 70 the purpose of the invention comprise nearly all soluble salts, especially normal salts, and preferably readily ionizable neutral salts, or similarly acting substances such as the sugars, especially cane sugar and the like.

75 Of the normal salts we have found the sulphates, chromates, chlorides and nitrates to be particularly useful. The sulphates have the strongest protective action and are followed in descending order of protective effect by the corresponding chromates, chlorides and nitrates, while acetates, oxalates and many other salts are also useful for the purpose, but not so effective. From our 80 researches it appears that in these classes of salts the protective effect varies almost in 85

55

60

65

70

75

80

85

90

95

100

versely as the molecular weight. Thus ammonium or lithium salts are most effective, followed by the corresponding salts of sodium, potassium, magnesium, aluminium and 5 so forth. As previously stated the use of neutral salts is preferred, though salts having an acid reaction may also be employed.

Substances such as cane sugar and the like are not so powerful in their protective action 10 as are many of the salts: thus for example the presence of 0.6 to 1% ammonium sulphate or about 2% sodium sulphate will protect the lustre of cellulose acetate artificial silk when boiled with water, while 10% cane sugar is required under the same conditions.

When the cellulose acetate artificial silk is subjected to the action of hot or boiling or other aqueous baths, capable of causing delustering thereof, the lustre may be protected 20 to any desired extent by the presence of one or more of the protecting agents or substances. The degree of protection will depend on the protecting agent employed and the concentration thereof, the nature and temperature of 25 the bath and the duration of the treatment. Thus for example only a slight degree of delustering is produced on subjecting cellulose acetate artificial silk to a 5% boiling solution of cane sugar for about 10 minutes or a 20% 30 solution of sodium chloride for about 30 minutes, the resultant product in these cases having a lustre approaching that of real silk, while the lustre is substantially unchanged on boiling cellulose acetate artificial silk for 35 about one hour with a 5% solution of ammonium sulphate or sodium sulphate.

For preventing or controlling the delustering action of moist steam we may apply the protecting agents or substances to the goods 40 in any suitable manner. For example the goods may be soaked in aqueous solution of the protecting agent, for instance ammonium sulphate, prior to exposure to the moist steam, the goods being dried prior to exposure if 45 desired.

The present invention affords valuable technical advantages in that it allows of preventing entirely or of regulating to any desired degree the delustering of goods consisting of or containing cellulose acetate artificial silk under the action of delustering agencies to which such goods are exposed in various processes or treatments to which they are commonly subjected in industry, for example dyeing, crêping, "crabbing", steaming, scouring and so forth. Especially we have found that the retarding or restraining influence of the 50 protecting agents is particularly useful with regard to "mixed" yarns, fabrics or materials 55 containing cellulose acetate artificial silk associated with wool or other fibres. It is often necessary to subject such mixed goods, particularly mixed goods containing wool and cellulose acetate artificial silk, to the action of hot or boiling baths and such treat-

ments often cause total or partial delustering of the cellulose acetate artificial silk. Thus for example in dyeing mixed yarns, fabrics or materials containing wool and cellulose acetate artificial silk, it is necessary to subject 70 the fabric to the action of hot or boiling baths, often for considerable time, to effect the dyeing of the wool, and in such cases the cellulose acetate artificial silk may be partially or often totally delustered. We have found that the 75 lustre of the cellulose acetate artificial silk can in such cases be protected or controlled to any desired degree by the presence of one or more of the protecting agents in the hot or boiling baths. Thus for example in dyeing 80 mixed goods composed of cellulose acetate artificial silk and wool, the presence of a protective salt such as referred to in the dye bath used for dyeing the wool portion, will allow 85 of preventing or regulating the delustering action of the dye bath as required: for instance as little as 20% relatively to the weight of the goods, of a salt such as ammonium sulphate will preserve the lustre of the cellulose acetate according to requirements.

It will be seen that the invention provides means not only of preventing partial or complete delustering of the cellulose acetate filaments etc. under the action of delustering agencies, but also of controlling or regulating the degree of partial or complete delustering to any desired extent, which is of advantage in many technical aspects. For example it is thus possible to modify the lustre to resemble that of natural silk or other fibres 100 or to any other desired degree for particular effects.

It will also be understood that not only can the invention be employed for preventing or regulating delustering of cellulose acetate artificial silk wholly or to any desired degree in processes or treatments to which goods consisting of or containing it are normally exposed in industry (e. g. dyeing, crêping, crabbing, steaming, scouring and so forth), 105 but that the invention can also be applied as an independent treatment to threads or goods consisting wholly or partly of cellulose acetate artificial silk for modifying the lustre of the cellulose acetate to any desired 110 controlled degree for the attainment of particular effects,—for instance to imitate natural silk or other fibres or other desired effects,—by subjecting the goods to the action of the delustering agencies and controlling their action by employment of protective salts or other protective agents as referred to. The term materials as used in the claims is to be interpreted as including threads, fabrics and other goods.

The phrase "hot aqueous medium" is used in the appended claims to include hot or boiling aqueous liquids, particularly such liquids as have a temperature of 90° C. or over, or moist steam, whether such agents are used 120

alone or in conjunction with other agents used in technical operations such as dyeing, creping, "crabbing", steaming, scouring, and so forth.

5 What we claim and desire to secure by Letters Patent is:—

1. In a process of treating a material containing lustrous cellulose acetate filaments with an agent which tends to delustre the material, conducting the treatment in the presence of a normal salt of neutral to acid reaction.

15 2. In a process of treating a material containing lustrous cellulose acetate filaments with a hot aqueous medium which tends to delustre the material, conducting the treatment in the presence of a normal salt of neutral to acid reaction.

20 3. In a process of treating a material containing lustrous cellulose acetate filaments with a hot aqueous medium which tends to delustre the material, conducting the treatment in the presence of a lustre protecting agent comprising a water soluble normal salt 25 of neutral to acid reaction dissolved to form a solution of a concentration effective to preserve the lustre of said materials at least in part.

4. In a process of treating a material containing lustrous cellulose acetate filaments with a hot aqueous medium which tends to delustre the material, conducting the treatment in the presence of a lustre protecting agent comprising a readily ionizable normal 35 salt of neutral to acid reaction, dissolved to form a solution of a concentration effective to preserve the lustre of said materials at least in part.

5. In a process of treating a material containing lustrous cellulose acetate filaments with a hot aqueous medium which tends to delustre the material, conducting the treatment in the presence of ammonium sulphate.

40 6. A process for treating a material containing lustrous cellulose acetate filaments for the purpose of modifying its lustre, which consists in submitting the material to the delustering action of a hot aqueous medium in the presence of a lustre-protecting agent in 45 a proportion lower than that necessary for maintaining the original lustre.

7. A process for treating a material containing lustrous cellulose acetate filaments for the purpose of modifying its lustre, which 55 consists in submitting the material to the action of a hot aqueous liquid in which is dissolved a lustre-protecting agent to form a solution of lower concentration than that necessary for maintaining the original lustre.

80 8. A process for treating a material containing lustrous cellulose acetate filaments for the purpose of modifying its lustre, which consists in submitting the material to the action of a hot aqueous liquid in which is dissolved a lustre-protecting saline agent to

form a solution of lower concentration than that necessary for maintaining the original lustre.

9. A process for treating a material containing lustrous cellulose acetate filaments for the purpose of modifying its lustre, which consists in submitting the material to the action of a hot aqueous liquid in which is dissolved a lustre-protecting agent comprising a normal salt of neutral to acid reaction to 70 form a solution of lower concentration than that necessary for maintaining the original lustre.

10. A process for treating a material containing lustrous cellulose acetate filaments for the purpose of modifying its lustre, which consists in submitting the material to the action of a hot aqueous liquid in which is dissolved a lustre-protecting agent comprising ammonium sulphate to form a solution of 80 lower concentration than that necessary for maintaining the original lustre.

In testimony whereof we have hereunto subscribed our names.

CHARLES WILFRED PALMER. 90  
STEPHEN MILLER FULTON.

70

75

80

85

90

95

100

105

110

115

120

125

130